

# UNITED STATES PATENT OFFICE.

RAYMOND F. BACON, OF PITTSBURGH, PENNSYLVANIA, ASSIGNOR TO METALS RECOVERY COMPANY, OF NEW YORK, N. Y., A CORPORATION OF MAINE.

## FLOTATION OF ORES.

1,235,954.

Specification of Letters Patent.

Patented Aug. 7, 1917.

No Drawing.

Application filed January 4, 1916. Serial No. 70,185.

To all whom it may concern:

Be it known that I, RAYMOND F. BACON, a citizen of the United States, residing at Pittsburgh, Allegheny county, State of Pennsylvania, have invented certain new and useful Improvements in Flotation of Ores; and I do hereby declare the following to be a full, clear, and exact description of the invention, such as will enable others skilled in the art to which it appertains to make and use the same.

This invention relates to the concentration of ores, and to the separation of metal constituents thereof from each other and from associated gangue, by a procedure which involves a fractional separation of the metal constituents by combined solution and sulfidation and by subsequent flotation treatment.

20 The common flotation processes of concentrating low grade sulfid ores involve the indiscriminate separation of sulfids from gangue. Where the sulfid particles are themselves superficially oxidized or coated 25 with an oxid film, it has been common practice to effect the flotation in the presence of an acid which will dissolve and thus remove such oxid films and leave the sulfid particles suitable for flotation. Metal constituents 30 thus dissolved are, however, lost, so far as the flotation procedure is concerned, and they can only be recovered by a subsequent treatment. The dilution of such solutions would often make recovery of the metal values therefrom impracticable.

It has heretofore been proposed to convert oxid ores into sulfids by treatment with hydrogen sulfid or soluble sulfids and by thereafter subjecting the ore to flotation; 40 but such procedures also commonly involve an indiscriminate separation of all sulfids formed from the gangue. Where the oxid or other non-sulfid constituents are present intimately blended with each other and 45 with the gangue, the sulfidized ore retains the ore constituents in a similar or corresponding state of combination.

It has further been proposed to separate 50 oxidized lead and zinc compounds in suspension in the presence of an acid by treatment with sulfureted hydrogen or a soluble sulfid, thereby coating only the lead with a layer of sulfid without converting the oxidized zinc into sulfid, the zinc oxid not being affected by the sulfid in an acid solution. The

thus partially sulfidized ore is subsequently subjected to flotation to recover the lead sulfid and leave the zinc behind in the pulp. With many ores such a proposal is not practicable because of the intimate blending of 60 the lead and zinc with each other and with the gangue, even in a finely crushed condition. Where the lead and zinc are thus blended, the particles will remain physically combined even after partial sulfidation, so 65 that a clear separation will be thus precluded.

The various procedures referred to above involve a preliminary crushing to effect physical separation of the gangue from the 70 ore. Where the ores are of such a nature that such physical separation cannot be effected by crushing, the separation is to that extent prevented or prejudiced. Similarly, the proposals to effect selective separation 75 of different sulfid constituents from each other or from oxidized constituents are subject to the limitation that where these constituents are intimately combined together in the same finely divided particles, their 80 separation is not practicable for the reason that the treated particles will still retain such constituents in a similar or corresponding state of combination.

The present invention relates to an improved method of effecting a selective or fractional separation and concentration of oxidized and other ores in a simple and improved manner, whereby the disadvantages 90 of prior proposals such as those referred to above are largely overcome or minimized. As distinguished from indiscriminate separations of sulfid constituents from gangue, the process of the present invention involves a selective or fractional separation of metal 95 constituents from each other which will be more clear and sharp, and which can be applied to ores incapable of satisfactory concentration and fractional separation by methods heretofore proposed. While all of 100 the proposals referred to above depend primarily upon the physical separation of the ore constituents from each other, the process of the present invention enables a separation of metal constituents from each other 105 where physical separation by crushing is not feasible.

According to the present invention, the oxidized or other ores containing metal constituents forming acid soluble and acid in- 110

soluble sulfids are treated with hydrogen sulfid or other soluble sulfid in the presence of a sufficient excess of acid to effect solution of the metal constituents forming acid soluble sulfids, whereby only the metal constituents are sulfidized which form acid insoluble sulfids. Thereby, the fractional sulfidation and solution is simultaneously effected, the acid dissolving certain metal constituents, and the sulfid converting other metal constituents into sulfids, so that, at the end of the process, the acid soluble metal constituents will be in solution, and the metal constituents forming acid insoluble sulfids will be converted, partially or completely, into sulfids. Furthermore, the disintegrating action of the acid in dissolving the acid soluble constituents tends to exert a further disintegrating action upon the ore particles, supplemental to the disintegrating action of the preliminary crushing of the ore.

The ores to be treated may be either of a sulfid or of an oxid or other non-sulfid nature, since the process is of more or less general application to ores containing metal constituents which are soluble in acids and form acid soluble sulfids and which also contain metal constituents forming insoluble sulfids. Where the ores are of an oxidized nature they can be treated according to the present invention after they have been preliminarily crushed or otherwise finely divided to effect more or less complete separation of the metal particles from the gangue.

In treating sulfid ores it may be necessary or advantageous to subject the ore to a partial or complete preliminary roast in order to thereby disintegrate the ore and convert the ore constituents into a form better adapted to the subsequent fractional separation. Thus, with zinc blend ores containing lead, the lead and zinc sulfids may be so intimately combined and blended with each other that it is impossible to effect a physical separation by any crushing procedure. This combination may even be so intimate that, upon treating with an acid and with the soluble sulfid simultaneously, the insoluble blend sulfid may prevent solution of the zinc from the oxidation of the ore particles. In such cases, it may be necessary to disintegrate the ore by a preliminary roast in order to facilitate extraction by the acid of the zinc or other acid soluble constituents forming acid soluble sulfids, at the same time that the soluble sulfid converts or completes the conversion of the lead into lead sulfid.

After a preliminary roast the zinc will be more readily extracted so that the combined extraction and sulfidation operation can proceed in a more advantageous manner. So also, where the zinc sulfid is present in sulfid ores in a form such that it can

be directly dissolved in the presence of the soluble sulfid, the preliminary roasting may not be necessary in order to obtain an effective separation. In all cases, however, the acid present should be of a sufficient amount and of a suitable strength to insure solution of the desired metal constituents forming acid soluble sulfids so that these metal constituents will be dissolved and held in solution at the same time that the soluble sulfid present is effecting the sulfidation. It will of course be understood, however, that the sulfidizing reaction may be completed before the extraction and solution of all acid soluble constituents, and that the combined solution and sulfidation accordingly may not be completed at the same time. The nature of the ore may make it advisable to continue the action of the acid for some time after the completion of the sulfidation, or in the presence of a small excess of the soluble sulfid, in order to complete or to increase the extraction of the acid soluble constituents.

In treating copper sulfid ores containing iron pyrites, or in treating mixed copper and iron sulfid ores such as chalcopyrite, with which iron sulfid is usually present, the ore may with advantage be first subjected to a preliminary roast at a suitable temperature to decompose the iron sulfid. The roasting may be conducted under conditions to prevent roasting of the copper sulfid although the sulfid may be oxidized to a greater or less extent. More or less silver, lead, zinc, etc., may also be present. The ore is next treated with a soluble sulfid such as hydrogen sulfid together with dilute sulfuric acid or other suitable acid in amount and of a strength sufficient to dissolve the iron and other constituents forming acid soluble sulfids; while the oxidized and dissolved copper will be sulfidized because of the insolubility of the copper sulfid in acids. This sulfidation, and the solution of the soluble constituents, will take place simultaneously.

With copper ores which are already in an oxidized state, such as the oxid or carbonate ores, the ores can be treated directly, in the form of the ore pulp or slimes or in suspension, with the soluble sulfid and the acid in suitable amount and of suitable strength, so that the formation of the copper sulfid and other acid insoluble sulfids, and the solution of the acid soluble constituents forming acid soluble sulfids, will take place at the same time, although as indicated above, the sulfidation may be complete before the solution, or may continue even after the solution, depending upon the relative amounts and strengths of the reagents employed.

After the sulfidation and solution reactions are completed, the ore is then subjected

to flotation to effect the removal of the sulfids. The flotation treatment may be an oil froth flotation, or it may be a flotation effected by aeration and froth formation without the use of oil, etc. The flotation treatment results in separation of the sulfids so that the remaining ore pulp contains the gangue together with the dissolved metal constituents. Thus, upon subjecting the 10 treated lead-zinc ores to flotation, the lead sulfid, or the partially sulfidized lead particles, will be removed, while the dissolved zinc will remain in solution in the ore pulp. Before the flotation, the excess acid present 15 may be partially neutralized, where the flotation treatment is of such a nature that an excess of acid would be prejudicial.

After the flotation treatment, and the separation of the sulfids, the dissolved metals 20 can be similarly separated from the gangue by a flotation treatment by first converting them into sulfids after neutralization of the excess acid. Thus ore pulps containing zinc in solution may be treated with an alkaline 25 sulfid or alkaline earth sulfhydrate, or with hydrogen sulfid and a neutralizing agent, to precipitate the zinc as zinc sulfid. By then subjecting the ore to a further flotation treatment the precipitated zinc sulfid 30 can be floated off and obtained in a form substantially free from lead.

In the treatment of pulp containing both copper and zinc, with the sulfid and acid, temporary precipitation of the zinc sulfid 35 may take place, particularly in dilute solutions, but this can be prevented by using a sufficient amount of acid. Also any precipitated zinc sulfid may further react with any dissolved and unsulfidized copper to 40 form copper sulfid, the zinc again going into solution. In such cases, and where a clear separation is not directly obtained, it may be advisable to continue the process until an equilibrium is reached so that the soluble 45 constituents may be dissolved and the insoluble sulfids may be produced.

In treating ores containing nickel and copper, together with other ore constituents, the nickel can be dissolved without dissolving the copper, or any dissolved copper 50 can be precipitated without precipitating the nickel as sulfid. After removal of the copper by flotation the nickel can subsequently be precipitated as sulfid by neutralizing the excess acid and by treatment with a soluble 55 sulfid, after which the precipitated nickel sulfid can itself be recovered by a further flotation treatment.

The soluble sulfid used for the sulfidizing 60 process may be hydrogen sulfid, or other soluble sulfid which will react in a similar manner. The alkaline sulfids will, in the presence of an excess of acid, be hydrolyzed into hydrogen sulfid so that they are the 65 equivalent of the hydrogen sulfid in the

procedure of the present invention where an excess of acid is present.

Similarly, after the acid insoluble sulfids have been removed, the excess acid can be neutralized and the acid soluble sulfids precipitated either by the use of an alkaline sulfid which will itself neutralize the excess acid, or by the use of hydrogen sulfid together with an added neutralizing agent. The alkaline sulfid may, for example, be 75 sodium sulfid or an alkaline earth sulfid or sulfhydrate, such as calcium sulfhydrate. Any excess of the hydrogen sulfid or soluble sulfid, which might be prejudicial to the flotation treatment, should be neutralized 80 before subjecting the ore to such treatment.

The acid used for dissolving the soluble constituents may be sulfuric acid of the strength used commercially for extracting ores, or it may be sulfur dioxid or mixtures 85 of sulfur dioxid with sulfur trioxid, which, when dissolved in the ore pulp, form sulfurous, or a mixture of sulfurous and sulfuric, acids. With some ores hydrochloric acid also can be used. The strength and 90 amount of the acid will necessarily vary somewhat with different ores, depending upon the strength and amount required for dissolving those metal constituents which 95 form acid soluble sulfids and which it is desired to retain in solution at the end of the sulfidizing process. Accordingly, it may be advisable to use an acid of somewhat greater strength, or in somewhat greater amount, than would otherwise be used for 100 extracting the ore if the sulfidizing agent were not simultaneously used. On the other hand, the amount of acid may be less than would be required for extracting the metal values if the sulfid were not also used as the 105 reagent, for the reason that the acid will dissolve only the metal constituents forming acid soluble sulfids, and not those forming acid insoluble sulfids.

By using sulfur dioxid as the acid, and 110 hydrogen sulfid as the sulfidizing agent, not only will the acid insoluble metal sulfids be precipitated, but colloidal sulfur will also be formed. The sulfur dioxid should, however, be used in considerable excess so that 115 it will effect the desired solution the same as would an excess of sulfuric acid, in order that all the soluble constituents may be dissolved and only the acid insoluble sulfids formed.

In my companion application Serial No. 36,698, filed June 28, 1915, I have described and claimed the treatment of non-sulfid ores, either simultaneously or successively, with sulfur dioxid and hydrogen sulfid, in 125 order to effect a sulfidizing of the ore and the formation of colloidal sulfur within the ore pulp. In said companion application I have also described and claimed the fractional or selective separation of metal con- 130

stituents from each other by such colloidal sulfur process. The claims of said application are, however, limited to a procedure wherein such colloidal sulfur is formed and made use of, for effecting the subsequent flotation; while in the present application the claims are drawn generically to the fractional or selective separation by the combined action of a soluble sulfid and an excess of any suitable acid sufficient in amount to effect solution of the soluble metal constituents at the same time that sulfidation of the constituents forming acid insoluble sulfids takes place. Accordingly, the colloidal sulfur process of said companion application may, by proper regulation and by effecting the combined sulfidation and solution simultaneously thereby, embody the generic features of novelty of the present invention; but the colloidal sulfur process specifically described and claimed in said companion application is of a more generic nature and is not limited to a fractional or selective separation in its broader aspect; and the colloidal sulfur process specifically claimed in said application is distinguished from the fractional separation process specifically claimed in the present application, in which sulfuric acid is used as the acid, and in which the formation of colloidal sulfur is not contemplated.

In my companion application, Serial No. 60,697, filed November 10, 1915, I have described and claimed a further method of effecting a fractional separation and concentration of ores by, first, dissolving the acid soluble constituents of the ore and thereby separating the same from the gangue, thereafter effecting a fractional precipitation of metal constituents forming acid insoluble sulfids from those forming acid soluble sulfids by treatment with hydrogen sulfid in the presence of a suitable excess of acid, and finally subjecting the resulting mixture to a flotation treatment. According to such process the solution of the metal constituents precedes the sulfidation treatment so that metal constituents forming acid insoluble sulfids will also be first dissolved if they are present in an acid soluble form. The process of the present invention is distinguished from such process by the fact that the solution and sulfidation take place simultaneously, instead of successively, so that metal constituents forming acid insoluble sulfids are produced directly without solution, except perhaps temporary or transitory solution, while the soluble constituents are dissolved in the presence of the sulfid which will not convert them into an acid insoluble form.

The method of the present invention is distinguished from proposals heretofore made to effect a fractional separation of oxidized ores by treating with sulfids in the

presence of acids which will prevent certain oxidized constituents from being sulfidized, by the fact that the acid is used, not in small amounts which will leave the soluble constituents present in the pulp in the form of their oxids, but in amounts sufficient to effect solution of these soluble oxidized constituents so that they are physically separated from the gangue and from the sulfidized particles. The particles which are already physically separated will of course also be dissolved, but the solution of the particles still mixed with or adhering to particles of gangue or particles containing constituents which will be sulfidized, results in removing the soluble constituents and thereby effecting a cleaner and more complete fractional separation. In other words, instead of leaving certain oxidized constituents, which will not sulfidize in the presence of acids, present in the ore pulp in an oxid and non-affected condition, the process of the present invention contemplates the solution of these constituents so that they are present at the end of the flotation treatment in a dissolved condition.

The flotation treatment, as already indicated, may be effected by aeration, with agitation, and resulting froth formation, or a small amount of oil can be beaten into the pulp together with the air, and a froth thus obtained.

In either case, the flotation is materially improved by the presence of the precipitated sulfids which are of a more or less colloidal nature than the naturally occurring sulfid constituents of the ore.

From the above description it will be noted that the invention is of more or less general application, both to the treatment of completely oxidized ores and to the treatment of partially oxidized ores, or even to some sulfid ores. In all cases the procedure involves the simultaneous sulfidation of constituents forming acid insoluble sulfids and solution of metal constituents forming acid soluble sulfids, and the subsequent removal of the sulfids formed by a flotation treatment. The treatment of oxid ores, however, is of particular value according to the present invention for the reason that the constituents forming acid soluble sulfids are more readily dissolved and for the further reason that the constituents forming acid insoluble sulfids are converted, superficially or completely, from the oxid to the sulfid form under conditions which make for a cleaner and more complete fractional separation. Furthermore, the production of the sulfids in the presence of the excess of acid, and from the oxidized ores which may be temporarily or transitorily dissolved during sulfidation, gives a sulfid which is readily separated by flotation treatment. In the treatment of oxid ores, and even in the treat-

ment of partially oxidized or sulfid ores, the use of sulfuric acid has important advantages for the reason that it does not prejudice the subsequent flotation and does not interfere with the sulfidation, and for the further reason that oxid ores readily dissolve in it as do also partially roasted or completely roasted ores which frequently contain considerable amounts of sulfates, and which thus promote the action of the sulfuric acid in dissolving the soluble constituents. The sulfuric acid can also be readily obtained from smelter fumes by oxidation so that it can be produced in amounts and concentration necessary for commercial operations, from the sulfid ores themselves.

I claim:

1. The method of concentrating ores and of effecting the separation of metal constituents forming acid soluble and acid insoluble sulfids from each other, which comprises subjecting the ores containing such constituents to the simultaneous action of hydrogen sulfid and of an acid in sufficient amount to effect solution of the acid soluble constituents forming acid soluble sulfids, and thereby effecting the fractional solution and extraction of such soluble constituents and the conversion of the constituents forming acid insoluble sulfids into sulfids, and finally subjecting the resulting mixture to a flotation treatment and thereby separating the insoluble sulfids from the ore pulp; substantially as described.
2. The method of concentrating ores and of effecting the separation of metal constituents forming acid soluble and acid insoluble sulfids from each other, which comprises subjecting the ores containing such constituents to the simultaneous action of hydrogen sulfid and of an acid in sufficient amount to effect solution of the acid soluble constituents forming acid soluble sulfids, and thereby effecting the fractional solution and extraction of such soluble constituents and the conversion of the constituents forming acid insoluble sulfids into sulfids, subjecting the resulting mixture to a flotation treatment and thereby separating the insoluble sulfids from the ore pulp; substantially as described.
3. The method of concentrating non-sulfid copper ores and of effecting the separation of copper from metals forming acid soluble sulfids, which comprises subjecting the ores to the simultaneous action of hydrogen sulfid and of an acid in sufficient amount to effect solution of the acid soluble constituents forming acid soluble sulfids, and there-

by effecting the fractional solution and extraction of such soluble constituents and the conversion of the non-sulfid copper constituents into sulfids, and finally subjecting the resulting mixture to a flotation treatment and thereby separating the insoluble copper sulfid from the ore pulp; substantially as described.

4. The method of concentrating zinc ores and of effecting the separation of zinc from metal constituents forming acid insoluble sulfids and from associated gangue, which comprises subjecting the ores to the simultaneous action of hydrogen sulfid and of an acid in sufficient amount to effect solution of the zinc, and thereby effecting the fractional solution and extraction of the zinc and the conversion of the constituents forming acid insoluble sulfids into sulfids, subjecting the resulting mixture to a flotation treatment and thereby separating the insoluble sulfids from the ore pulp, subsequently precipitating the zinc as sulfid by neutralizing the excess acid and treating with a suitable sulfid, and finally subjecting the mixture to a further flotation treatment and thereby separating the precipitated zinc sulfid from the ore pulp; substantially as described.

5. The method of concentrating ores containing iron pyrites and of effecting the separation of metal constituents forming acid insoluble sulfids from the iron pyrites, which comprises subjecting such ore to a preliminary roast to convert the iron pyrites into an acid soluble form, subjecting the roasted ore to the simultaneous action of hydrogen sulfid and of an acid in sufficient amount to prevent conversion of the iron into sulfid, and thereby effecting the conversion of the constituents forming acid soluble sulfids into sulfids, and finally subjecting the resulting mixture to a flotation treatment and thereby separating the insoluble sulfids from the ore pulp; substantially as described.

6. The method of concentrating sulfid ores containing lead and zinc and of effecting the separation of the lead and zinc from each other, which comprises roasting the ore to convert the zinc into a soluble form, subjecting the roasted ore to the simultaneous action of hydrogen sulfid and of an acid in sufficient amount to effect solution of the zinc, and thereby effecting the fractional solution and extraction of the zinc and the conversion of the lead into sulfid, subjecting the resulting mixture to a flotation treatment and thereby separating the lead sulfid and other acid insoluble sulfids from the ore pulp, subsequently precipitating the zinc as sulfid, and again subjecting the mixture to a flotation treatment and thereby separating the precipitated zinc sulfid from the ore pulp; substantially as described.

7. The method of concentrating ores and

of effecting the separation of metal constituents forming acid soluble and acid insoluble sulfids from each other, which comprises subjecting the ores containing such 5 constituents to the simultaneous action of hydrogen sulfid and of sulfuric acid in amount sufficient to effect solution of the acid soluble constituents forming acid soluble sulfids, and thereby effecting the fractional 10 solution and extraction of such soluble constituents and the conversion of the constituents forming acid insoluble sulfids into sulfids, and finally subjecting the resulting mixture to a flotation treatment and 15 thereby separating the insoluble sulfids from the ore pulp; substantially as described.

8. The method of concentrating zinc ores and of effecting the separation of the zinc from metal constituents forming acid 20 insoluble sulfids, which comprises subjecting the ores to the simultaneous action of hydrogen sulfid and of sulfuric acid in sufficient amount to dissolve the zinc as sulfate and to prevent precipitation of zinc sulfid, 25 and thereby effecting fractional solution and extraction of the zinc and the conversion of the constituents forming acid insoluble sulfids into sulfids, subjecting the resulting mixture to a flotation treatment and thereby 30 separating the insoluble sulfids from the ore pulp, subsequently precipitating the zinc as sulfid by neutralizing the excess sulfuric acid and treating with a suitable sulfid; and finally subjecting the resulting mixture to a further flotation treatment and 35 thereby separating the zinc sulfid from the ore pulp; substantially as described.

9. The method of concentrating sulfid ores containing lead and zinc and of effecting the separation of the lead and zinc from each other, which comprises subjecting the ore to a sulfatizing roast, subjecting the roasted ore to the simultaneous action of hydrogen sulfid and of sulfuric acid in amount sufficient to effect solution of the zinc as sulfate, and thereby effecting a fractional 40 solution and extraction of the zinc as zinc sulfate and the conversion of the lead into sulfid, and finally subjecting the resulting mixture to a flotation treatment 45 and thereby separating the lead sulfid and other acid insoluble sulfids from the ore pulp; substantially as described.

10. The method of concentrating sulfid ores containing iron pyrites, and lead, copper and zinc constituents, and of effecting the separation of the lead and copper from the zinc and from the iron pyrites, which comprises subjecting the ore to a preliminary roast to convert the iron pyrites into an acid soluble form, subjecting the roasted ore to the simultaneous action of hydrogen sulfid and of a sufficient amount of acid to effect the solution of the zinc and iron, and thereby effecting the fractional solution and 55 extraction of the zinc and iron and the conversion of the lead and copper into sulfids, and finally subjecting the resulting mixture to a flotation treatment and thereby separating the lead and copper sulfids from the ore 60 pulp; substantially as described.

In testimony whereof I affix my signature.

RAYMOND F. BACON.